

April 22, 1952

F. E. NEWMAN

2,594,061

PLATING BARREL

Filed Oct. 25, 1949



INVENTOR.  
FERRIS E. NEWMAN  
BY  
*Robert J. Patterson*  
ATTORNEY

## UNITED STATES PATENT OFFICE

2,594,061

## PLATING BARREL

Ferris E. Newman, New Haven, Ind., assignor to  
 United States Rubber Company, New York,  
 N. Y., a corporation of New Jersey

Application October 25, 1949, Serial No. 123,441

9 Claims. (Cl. 259—89)

1

This invention relates to plating barrels and more particularly to a non-metallic plating barrel which is far superior to non-metallic plating barrels heretofore employed.

In plating small metal parts, in order to save considerable handling, it has become customary in the art to place the parts in a perforated non-metallic barrel for transfer through the cleaning and plating baths. Prolonged exposure to strong acid pickling solutions and to alkali cleaners at temperatures ranging as high as 200° F. places considerable strain on the barrel. Parts of the barrel all of which must be non-metallic include a large diameter gear (usually of the order of 16" in diameter), bearings and structural panels. A number of non-metallic materials have been used for the fabrication of such barrels but all of them have serious shortcomings. Hard rubber has been used but it is brittle and has extremely poor resistance to elevated temperatures. It has also been proposed to make the barrels from laminates composed of layers of cloth bonded together with phenolic resins or with melamine resins. However, both of these resin-cloth laminates have poor abrasion resistance and the phenolic laminates rapidly disintegrate in alkali and the melamine laminate rapidly disintegrates in acid. The prior art barrels have also been subject to other disadvantages including the high cost of manufacture due to the difficulty of working with the materials heretofore used in construction of plating barrels.

For these reasons, plating barrels heretofore available have not stood up satisfactorily in service. For a long time workers in the art have been aware of the shortcomings of the available non-metallic plating barrels but have been unable to remedy these shortcomings.

I have now discovered that a plating barrel far superior to those heretofore available may be formed from a heat-cured composition comprising a cashew nut shell oil-modified phenol-aldehyde resin which is convertible under the action of heat and an intermixed hardening agent to insoluble, infusible form, a hardening agent for the resin, typically and almost invariably hexamethylenetetramine, a rubbery copolymer of butadiene and acrylonitrile, and diatomaceous earth. The plating barrels of my invention are superior to prior plating barrels in the following respects: hot acid resistance, hot alkali resistance, impact strength, abrasion resistance, structural strength at 200 F., and ease of fabrication. As a result the plating barrels of my invention exhibit an extremely long service life even under the most severe service conditions and greatly reduce the cost of plating operations.

2

In the accompanying drawings:

Fig. 1 is a side elevation, partly broken away in section, of a typical plating barrel made in accordance with my invention.

Fig. 2 is a partial end view of the plating barrel shown in Fig. 1, taken on the line 2—2 of Fig. 1.

Fig. 3 is an enlarged section through a laminated panel which may be employed in a modification.

In Figs. 1 and 2 of the drawings, the barrel of my invention is shown as embodying a pair of circular end members or cylinder heads 1, between which are arranged six foraminous panels 2 which have reduced end portions 3 entering corresponding recesses in the inner faces of end members 1 and reduced side portions 4 which enter corresponding recesses in longitudinal rail members 5 which are of square cross-section. Rail members 5 and end members 1 are fixedly secured together in permanent relationship by means of studs 6 which pass through end members 1 into the ends of rail members 5. The end portions 7 of rail members 5 are reduced in size and circular in cross-section and enter corresponding circular recesses in end members 1, clearance being provided between the ends of rail members 5 and the bottoms of the receiving recesses in end members 1 so that it is possible by means of studs 6 to draw the shoulders of rail members 5 into tight engagement with end members 1. The arrangement shown permits the ends 1, rails 5 and panels 2 to be assembled into permanent tight relationship. It will be understood that in accordance with customary practice in the art, one of the panels 2 is made quickly detachable for charging and discharging the barrel. The detachable panel 2 is not illustrated because its construction is well known to the art.

Panels 2 are provided with perforations 8 which allow the cleaning and plating solutions free access into and egress from the interior of the barrel.

The following provision is made for mounting the barrel for rotation. Coaxially with the barrel at each end thereof there is provided an annular hub 9 which is tightly secured to the adjacent end member 1 by means of studs 10. Within each of hubs 9 there is disposed a floating, freely rotatable, sleeve bearing 11 which freely rotatably engages hub 9 and the stationary supporting sheave 12. Sheave 12 is fixedly secured to the conventional rubber-covered metal supporting arm 13 by means of studs 14. It will be understood that the construction of each end of the barrel is identical and that each end of the barrel is supported in an identical manner. As is conventional, supporting arms 13 form part of

a yoke (not shown) which enables the barrel assembly to be moved easily from one tank to another. Details of the yoke are not shown because it is conventional in the plating barrel art.

The barrel of my invention is driven in the following manner: surrounding the hub 9 and mounted coaxially with the barrel at one end thereof there is provided a driving gear 15 which is fixedly secured to the adjacent end 1 of the barrel by studs 16, spacers 17 serving to space the gear a suitable distance from the end 1. It will be understood that the gear 15 is driven by a stainless steel driving gear (not shown) which is conventionally provided in the assembly in which the plating barrel is placed during operation.

In the modified form of panel 2a shown in Fig. 3, a laminated structure is employed, the major proportion of the thickness of the panel constituting a core 20 to which facings 21 are laminated. Preferably such a laminated panel is made by assembling the uncured laminae and curing them together under heat and pressure whereby there is coalescence at the interface. Use of a laminated structure as shown in Fig. 3 enables the major portion thereof, i. e., the core 20, to be formed from the above composition with the components in proportions imparting high strength, great stiffness, and freedom from creep at temperatures up to 200° F., and the facings 21 to be made of the material with relative proportions of the three major ingredients such as to impart high abrasion resistance.

An important novel feature of the barrel of my invention is that it is constructed throughout of the above-mentioned heat-cured composition of a cashew nut shell oil-modified phenol-aldehyde resin, a hardening agent therefor, a rubbery copolymer of butadiene and acrylonitrile, and diatomaceous earth. I have found it possible to make every part of the barrel including not only the end members 1, the panels 2 and the rails 5 but also the studs 6, the hubs 9, the studs 10, the bearings 11, the sheaves 12, the studs 14, the gear 15, the studs 16 and the spacers 17 from such a heat-cured composition. The result is that a barrel having remarkably long service life is obtained. In addition, the barrel is easily manufactured because of the easy machining properties of the composition.

It will be understood that with the construction shown in the drawings, the cleaning or plating liquid can pass freely through the center of the hollow bearing collar or sheave 12 and has free access to the bearing assembly but does no harm because it can touch no exposed metal.

The floating bearing construction of my invention is highly advantageous because it is adapted to very long life. There is plastic-to-plastic movement in the bearing mechanism and this is much superior to a bearing in which metal is substituted for any part of the bearing structure shown. The known non-metallic plating barrels available to the art heretofore have in recent years been provided with a floating bearing made of nylon but such bearings are extremely expensive and must be replaced very frequently. In contrast, the bearing construction of my invention is cheap and long-lived.

In the usual practice of my invention, all parts of the plating barrel as well as the associated parts, viz., the hubs 9, gear 15, bearings 11, sheaves 12, studs 6, 10, 14 and 16 and spacers 17 are formed of the above-identified composition wherein the relative proportions are such that

the rubbery copolymer of butadiene and acrylonitrile ranges from 30 to 60%, the cashew nut shell oil-modified phenol-aldehyde resin correspondingly ranges from 70 to 40% and the diatomaceous earth ranges from 30 to 55%, these percentages being by weight based on the sum of the weights of the rubbery copolymer and the resin. As will presently appear, however, I prefer to employ varying proportions of the three ingredients in constructing the various parts of the plating barrel assembly.

Thus I prefer to form the end members 1 and the panels 2 or the cores 20 of the panels 2a from the above composition in relative proportions of from 30 to 40% of the rubbery copolymer and correspondingly from 70 to 60% of the resin, and from 30 to 40% of diatomaceous earth. Use of these proportions gives a composition having good abrasion-resistance, high modulus, and excellent dimensional and structural stability.

I prefer to form the rails 5, hubs 9, bearings 11 and sheaves 12 from the above composition in relative proportions of from 30 to 45% of the rubbery copolymer and correspondingly from 70 to 55% of the resin, and from 30 to 45% of diatomaceous earth. These proportions impart freedom from creep at elevated temperatures, good structural strength at such temperatures, and also (this being important in the case of the bearings 11) good resistance to wearing upon prolonged plastic-to-plastic movement.

Where a laminated type of panel 2a is employed, I prefer to form the facings 21 from the above composition in relative proportions of from 45 to 60% of the rubbery copolymer and correspondingly from 55 to 40% of the resin, and from 40 to 55% of diatomaceous earth. Facings formed of such a composition are unusually resistant to abrasion.

I prefer to form the driving gear 15 from a composition embodying from 45 to 60% of the rubbery copolymer and correspondingly from 55 to 40% of the resin, and from 40 to 55% of diatomaceous earth. A gear so made displays unusual resistance to the abrasion of the mating stainless steel driving gear and excellent resistance to accidental impact in moving the barrel from tank to tank.

I prefer to form the studs 6, 10, 14 and 16 from the above composition in relative proportions of from 35 to 40% of the rubbery copolymer and correspondingly from 65 to 60% of the resin, and from 35 to 40% of diatomaceous earth. Studs formed from these proportions are resistant to creep at elevated temperatures and strong enough to enable the parts secured thereby to be tightly drawn together into permanent assembly and without shearing under the action of the wrench or driving tool.

Spacers 17 are preferably formed from the same composition as studs 6, 10, 14 and 16.

I have found that manufacture of the various parts of the plating barrel and associated parts in the assembly from the various compositions just described considerably enhances the life of the plating barrel and its utility because each of the compositions described imparts particular properties required of each of the various parts.

The composition of matter from which the parts of the plating barrel of my invention are formed, can be made by first preparing a homogeneous mixture of a cashew nut shell oil-modified phenol-aldehyde resin, a hardening agent for said resin, particularly a methylene-yielding sub-

stance, especially hexamethylenetetramine, which

is capable of advancing the resin to the insoluble, infusible stage under the action of heat, a rubbery copolymer of butadiene and acrylonitrile, viz., synthetic rubber of the type known as Buna N and as GR-A, and diatomaceous earth. Upon shaping such a mixture to the desired form and heat-curing it, the shaping and curing typically being effected either by preforming the powdered mixture by pressure alone, followed by molding of the preform under heat and pressure, or by molding of the mixture directly under heat and pressure, the mixture is converted to a material having an unusual combination of physical properties.

Any cashew nut shell oil-modified phenol-aldehyde resin capable of being advanced to insoluble, infusible form under the action of heat and a hardening agent, such as hexamethylenetetramine, may be employed in the practice of my invention. Such resins are extremely well-known, being available commercially. An example of such a resin is that known in the trade as Durez No. 12686. Another example is Durez No. 12687 which is a mixture of 92 parts of the resin sold as Durez No. 12686 and 8 parts of hexamethylene-tetramine. Still other examples of such resins containing hexamethylenetetramine as the hardening agent are the resins known in the trade as Varcum 9820 and Varcum 9831. Such resins may be made in the manner disclosed in detail hereinafter.

As is well-known, cashew nut shell oil, which is obtained from the outer shell of the cashew nut, is composed largely of anacardic acid which upon heating is decomposed and converted to a long-chain unsaturated phenol, known as cardanol, which has a 7-tetradecenyl side-chain,



in the position meta to the hydroxyl group on the benzene ring. While cashew nut shell oil itself may be used as obtained from the shell, I prefer to use the oil which has been heated to convert it to the phenol just described by decarboxylation in the well-known manner.

The lower molecular weight phenol used in conjunction with the cashew nut shell oil in making the resin is either a monohydric or a polyhydric, preferably the former, monocyclic phenol which contains no substituents on the benzene ring other than hydrogen, hydroxyl groups and lower alkyl side-chains. Examples of such lower molecular weight phenols are phenol itself, and its homologues, such as ordinary cresylic acid which is a mixture containing the three isomeric cresols, the xylenols, etc. Instead of a monohydric phenol, a polyhydric phenol, such as resorcinol, may be used.

While the proportion of cashew nut shell oil used in making the phenolic resin may vary widely, I prefer to use it in an amount ranging from 3 to 12 mole per cent based on the sum of the moles of the cashew nut shell oil and the lower molecular weight phenol. If less than 3 mole per cent of cashew nut shell oil is used, the phenolic resin may be unduly brittle and consequently may impart objectionable brittleness to the cured blends with the Buna N and the diatomaceous earth. Within the broad purview of my invention the molar proportion of cashew nut shell oil used in making the resin may be outside the range given; thus it may range from 2 mole per cent up to 50 mole per cent based on the sum of the moles of the cashew nut shell oil and the phenol.

Ordinary phenol is the preferred phenol for making the resin. As ordinary phenol is replaced by cresol, there is a tendency for the resin obtained to become softer with a consequent lowering of the hardness of the cured product.

The resin is typically made by heating a mixture of the lower molecular weight phenol, the cashew nut shell oil (either as such or in the de-carboxylated form) and an aldehyde, typically formaldehyde, in the presence of a suitable resin-forming catalyst, usually an acid, such as an inorganic acid, e. g., sulfuric or hydrochloric acid, or an acid-reacting material, as zinc chloride, to an oil-soluble stage. During the final stage of the reaction, the resin is advanced to the desired state at which it is still convertible to insoluble, infusible form under the action of heat and a hardening agent, and volatile materials are removed therefrom, these objects preferably being accomplished simultaneously by passing superheated steam through the charge until the residual mixture has reached the desired temperature, say 150° C. to 225° C. The residual mixture is then dumped from the kettle and allowed to cool. The cooled resin is then blended with the Buna N and the diatomaceous earth in the manner described hereinafter.

The resins used in accordance with the present invention are characterized by being completely miscible in all proportions with butadiene-acrylonitrile rubbery copolymers of relatively high acrylonitrile content, i. e., containing from 35 to 45%, or even more, of combined acrylonitrile.

As the rubbery copolymer of butadiene and acrylonitrile used in the practice of the present invention, I much prefer to employ those rubbery copolymers containing a relatively high proportion of combined acrylonitrile, say from 35 to 45%, because these rubbery copolymers are completely compatible with the resin whereas rubbery copolymers of lower acrylonitrile content often tend to exhibit somewhat diminished compatibility resulting in somewhat poorer physical properties. A butadiene-acrylonitrile rubbery copolymer which gives unusually satisfactory results in the present invention is that known commercially as Hycar OR-15 which contains about 42% combined acrylonitrile. Another material which gives very excellent results is that known as Perbunan 35 which contains about 35% combined acrylonitrile.

Less preferably, I may use rubbery copolymers of butadiene and acrylonitrile containing less than 35% combined acrylonitrile, say from 15% up to 35%. Examples of such copolymers are those known commercially as Perbunan 26 and Perbunan 18 which contain approximately 26 and 18% acrylonitrile, respectively. As the combined acrylonitrile content is lowered, the compatibility with the phenolic resin tends to progressively decrease and the physical properties of the product tend to be progressively poorer.

The third major component of the composition used in the practice of the present invention is diatomaceous earth. Any of the forms of granular or powdered diatomaceous earth commonly available commercially may be used in the practice of my invention. Usually the diatomaceous earth has a relatively small particle size. Generally it is so fine that substantially all of it will pass a 100 mesh sieve. Usually the particle size of this material will cover a range of from as large as 100 microns down to particles too small to be seen. I have obtained very

satisfactory results using the diatomaceous earth known in the trade as "Dicalite 14W," also known as grade L, put out by the Dicalite Company.

In addition to the three principal components mentioned above, the composition used in the plating barrels of my invention also contains a hardening agent, preferably hexamethylene-tetramine or its known equivalent, in amount sufficient to advance the resin to hard, infusible, insoluble condition during curing at elevated temperatures. Typically, the amount of hardening agent required to accomplish this is relatively small in proportion to the other components. Usually the proportion of this hardening agent will range from 5 to 10% by weight based on the resin alone.

The composition may also contain small amounts of other suitable materials such as mold lubricants, pigments and coloring agents to give the desired color, anti-oxidants for the rubber, etc. If desired, vulcanizing agents, such as sulfur, and other vulcanizing ingredients, such as the usual vulcanization accelerators and activators, may also be present although they are not necessary and in some cases it is believed that slightly better results are obtained without the use of such rubber vulcanizing agents and ingredients.

The foregoing ingredients are commingled together to form a uniform homogeneous mixture in any suitable manner, typically by means of a Banbury mill or a roll mill of the type used for compounding rubber. The resulting mixture is sheeted out, as on a rubber calender, and is allowed to cool. It is then comminuted, as by chopping or grinding, to a powdered or granulated material of suitable size for use in making preforms or for use directly as a molding powder. It is usually preferable to refrigerate the sheeted stock to facilitate the chopping or grinding. Typically, the stock is cooled to 35° F., or below, for this purpose. A conventional rotary knife machine may be used for grinding or chopping the mixture.

The resulting granular or powdered material may then be preformed with pressure but without heat to give preforms from which finished articles can be molded by subjecting the preforms to heat and pressure to give the desired shape and cause the material to flow together and thus coalesce to a continuous integral form and at the same time to cause the resin content of the mixture to advance to insoluble, infusible condition and to cure the mixture. The granular or powdered material exhibits the very advantageous property that upon being subjected to moderate pressure (without heat) the particles coalesce to such an extent that there is obtained a preform which retains its integrity even under conditions of plant handling. In this way many savings can be effected.

Instead of making preforms, the particulate molding material can be loaded directly into the molding equipment. Whether preformed or not, the material can be molded by any of the conventional molding methods such as compression molding or transfer molding or by simple placement into a mold cavity between heated platens and subjection to an elevated temperature, say of the order of 300 to 350° F., and to pressure, say of the order of 100 to 4000 lbs. per square inch, to form a cured sheet, slab or other article. A marked advantage of the mixture is that extremely high molding pressures such as are commonly required with the conventional phenolic molding material, viz., pressures of the order of

2000 lbs. per square inch and over, are not required. Pressures of the order of 200 to 1500 lbs. per square inch are ample for molding the material of the present invention. Another advantage is that the material cures very rapidly so that the productivity of the molding equipment is high.

Regardless of the method of forming or shaping the mixture, the molding temperatures, pressure and time should be such that the mixture flows properly together to give a solid, uniform, integral molded article and that the phenolic resin is converted to the insoluble, infusible state. The curing time required may vary widely, say from ten minutes to four hours, depending upon many factors, such as whether or not preforming was used, the thickness of the molding, etc. There seems to be no limit on curing time beyond which the properties of the material deteriorate. There is however, a minimum time, namely, the time required for complete curing; at the end of this time the physical properties of the mixture have reached their maximum.

The material of the present invention can be molded to very close tolerances. This makes it possible, for example, to mold the material directly into such articles as gears 15 with the teeth formed in the mold and with no need for subsequent machining. This is in marked contrast to prior art materials from which silent gears have, of necessity, been made by first molding a blank and then machining this blank into the finished gear. It will be understood, however, that if desired, the material of the present invention can be molded into sheets or blanks which can then be machined to give the desired articles.

The following illustrates typical formulae used for the various parts of the plating barrel of my invention.

|                         | Composition A | Pounds |
|-------------------------|---------------|--------|
| Hycar OR-15.....        |               | 16     |
| Durez 12837.....        |               | 30     |
| Dicalite 14W.....       |               | 14     |
| Zinc stearate.....      |               | 0.25   |
| Anti-oxidant.....       |               | 0.3    |
| Wax.....                |               | 0.25   |
| Iron oxide pigment..... |               | 3.0    |

This composition when mixed and processed as described above is very satisfactory for the construction of end members 1, panels 2, rails 5, hubs 9, bearings 11, and sheaves 12.

|                         | Composition B | Pounds |
|-------------------------|---------------|--------|
| Hycar OR-15.....        |               | 10.80  |
| Durez 12837.....        |               | 16.56  |
| Dicalite 14W.....       |               | 10.00  |
| Wax.....                |               | 0.27   |
| Anti-oxidant.....       |               | 0.18   |
| Iron oxide pigment..... |               | 3.12   |

This material is very satisfactory as a material from which to make end members 1, panels 2, rails 5, hubs 9, bearings 11, sheaves 12, studs 6, 10, 14 and 16 and spacers 17.

|                    | Composition C | Pounds |
|--------------------|---------------|--------|
| Hycar OR-15.....   |               | 24     |
| Durez 12837.....   |               | 18     |
| Dicalite 14W.....  |               | 18     |
| Zinc stearate..... |               | 0.3    |
| Anti-oxidant.....  |               | 0.3    |

This composition is usually suitable for the manufacture of driving gear 15 and facings 21 of

panels 2a. Where facings 21 of this composition are provided, the core 20 may be formed of Composition A above for good stiffness.

| Composition D           | Pounds |
|-------------------------|--------|
| Hycar OR-15.....        | 20     |
| Durez 12687.....        | 20     |
| Dicalite 14W.....       | 20     |
| Zinc stearate.....      | 0.3    |
| Iron Oxide Pigment..... | 1.8    |
| Anti-oxidant.....       | 0.3    |

This material is extremely well suited for the fabrication of gear 15.

| Composition E           | Pounds |
|-------------------------|--------|
| Hycar OR-15.....        | 18     |
| Durez 12687.....        | 24     |
| Dicalite 14W.....       | 18     |
| Zinc stearate.....      | 0.3    |
| Anti-oxidant.....       | 0.3    |
| Iron Oxide Pigment..... | 1.8    |

This composition is very suitable for the manufacture of rails 5, hubs 9, bearings 11, and sheaves 12.

From the foregoing description it will be seen that the present invention provides a plating barrel which effectively overcomes the disadvantages of prior art non-metallic plating barrels. The barrels of my invention are simple and easy to construct and are rugged and long-lived in service. They withstand the action of cleaning and plating solutions remarkably well even at elevated temperature as high as 200° F., and also resist abrasion and impact. The excellent machining characteristics of the material from which they are formed and its relatively low cost are unusually advantageous. The plating barrels of my invention are highly inert chemically and electrically so that no problem of contamination thereby is presented. Numerous other advantages of the plating barrels of my invention will be apparent to those given in the art.

The composition of matter described herein is disclosed and claimed in my copending application Serial No. 98,153 filed June 9, 1949. Silent gears made of this composition are described and claimed in my copending application Serial No. 98,152 filed on the same day.

Having thus described my invention what I claim and desire to protect by Letters Patent is:

1. A plating barrel comprising a pair of end members forming the ends of the barrel, a plurality of foraminous panels held longitudinally between said end members and forming the sides of the barrel, and a plurality of longitudinal rail members between said panels, said parts being composed of a heat-cured composition comprising a cashew nut shell oil-modified phenol-aldehyde resin convertible to insoluble, infusible form under the action of heat and a hardening agent, a methylene-yielding hardening agent for said resin, a rubbery copolymer of butadiene and acrylonitrile, and diatomaceous earth, the relative proportions being as follows: in said end members and in at least a major proportion of the thickness of said panels from 30 to 40% of said copolymer and correspondingly from 70 to 60% of said resin, and from 30 to 40% of diatomaceous earth; in said rail members from 30 to 45% of said copolymer and correspondingly from 70 to 55% of said resin, and from 30 to 45% of diatomaceous earth; said percentages being by weight based on the sum of said copolymer and said resin.

2. A plating barrel comprising a pair of end members forming the ends of the barrel, a plurality of foraminous panels held longitudinally between said end members and forming the sides of the barrel, a plurality of longitudinal rail members between said panels, and a floating freely rotatable sleeve bearing located at each end of the barrel coaxially therewith centrally of said end members, said parts being composed of a heat-cured composition comprising a cashew nut shell oil-modified phenol-aldehyde resin convertible to insoluble, infusible form under the action of heat and a hardening agent, a methylene-yielding hardening agent for said resin, a rubbery copolymer of butadiene and acrylonitrile, and diatomaceous earth, the relative proportions being as follows: in said end members and in at least a major portion of the thickness of said panels from 30 to 40% of said copolymer and correspondingly from 70 to 60% of said resin, and from 30 to 40% of diatomaceous earth; in said rail members and in said bearings from 30 to 45% of said copolymer and correspondingly from 70 to 55% of said resin, and from 30 to 45% of diatomaceous earth, said percentages being by weight based on the sum of said copolymer and said resin.
3. A plating barrel comprising a pair of end members forming the ends of the barrel, a plurality of foraminous panels held longitudinally between said end members and forming the sides of the barrel, a plurality of longitudinal rail members which with said end members support said panels, a floating freely rotatable sleeve bearing located at each end of the barrel coaxially therewith centrally of said end members, and a hub located at each end of the barrel coaxially therewith centrally of said end members, said hubs being fixedly connected to said end members, said bearings freely rotatably floating inside said hubs in frictional engagement therewith, said parts being composed of a heat-cured composition comprising a cashew nut shell oil-modified phenol-aldehyde resin convertible to insoluble, infusible form under the action of heat and a hardening agent, a methylene-yielding hardening agent for said resin, a rubbery copolymer of butadiene and acrylonitrile, and diatomaceous earth, the relative proportions being as follows: in said end members and in at least a major proportion of the thickness of said panels from 30 to 40% of said copolymer and correspondingly from 70 to 60% of said resin, and from 30 to 40% of diatomaceous earth; in said rail members, said bearings and said hubs from 30 to 45% of said copolymer and correspondingly from 70 to 60% of said resin, and from 30 to 45% of diatomaceous earth; said percentages being by weight based on the sum of said copolymer and said resin.
4. A plating barrel comprising a pair of end members forming the ends of the barrel, a plurality of foraminous panels held longitudinally between said end members and forming the sides of the barrel, a plurality of longitudinal rail members between said panels, and a driving gear fixedly connected to one of said end members coaxially with the barrel, said parts being composed of a heat-cured composition comprising a cashew nut shell oil-modified phenol-aldehyde resin convertible to insoluble, infusible form under the action of heat and a hardening agent, a methylene-yielding hardening agent for said resin, a rubbery copolymer of butadiene and acrylonitrile, and diatomaceous earth, the relative

proportions being as follows: in said end members and in at least a major proportion of the thickness of said panels from 30 to 40% of said copolymer and correspondingly from 70 to 60% of said resin and from 30 to 40% of diatomaceous earth; in said rail members from 30 to 45% of said copolymer and correspondingly from 70 to 55% of said resin, and from 30 to 45% of diatomaceous earth; in said gear from 45 to 60% of said copolymer and correspondingly from 55 to 40% of said resin, and from 40 to 55% of diatomaceous earth; said percentages being by weight based on the sum of said copolymer and said resin.

5. A plating barrel comprising a pair of end members forming the ends of the barrel, a plurality of foraminous panels held longitudinally between said end members and forming the sides of the barrel, a plurality of longitudinal rail members which with said end members support said panels, a floating freely rotatable sleeve bearing located at each end of the barrel coaxially therewith centrally of said end members, a hub located at each end of the barrel coaxially therewith centrally of said end members, said hubs being fixedly connected to said end members, said bearings freely rotatably floating inside said hubs in frictional engagement therewith, and a driving gear fixedly connected to one of said end members, said driving gear being mounted coaxially with said barrel and surrounding one of said hubs, said parts being composed of a heat-cured composition comprising a cashew nut shell oil-modified phenol-aldehyde resin convertible to insoluble, infusible form under the action of heat and a hardening agent, a methylene-yielding hardening agent for said resin, a rubbery copolymer of butadiene and acrylonitrile, and diatomaceous earth, the relative proportions being as follows: in said end members and in at least a major proportion of the thickness of said panels from 30 to 40% of said copolymer and correspondingly from 70 to 60% of said resin, and from 30 to 40% of diatomaceous earth; in said rail members, said bearings and said hubs from 30 to 45% of said copolymer and correspondingly from 70 to 55% of said resin, and from 30 to 45% of diatomaceous earth; in said gear from 45 to 60% of said copolymer and correspondingly from 55 to 40% of said resin and from 40 to 55% of diatomaceous earth; said percentages being by weight based on the sum of said copolymer and said resin.

6. A plating barrel comprising a pair of end members forming the ends of the barrel, a plurality of foraminous panels held longitudinally between said end members and forming the sides of the barrel, a plurality of longitudinal rail members between said panels, said rail members having recesses into which said panels extend, and studs securing said rail members to said end members, said parts being composed of a heat-cured composition comprising a cashew nut shell oil-modified phenol-aldehyde resin convertible to insoluble, infusible form under the action of heat and a hardening agent, a methylene-yielding hardening agent for said resin, a rubbery copolymer of butadiene and acrylonitrile, and diatomaceous earth, the relative proportions being as follows: in said end members and in at least a major proportion of the thickness of said panels from 30 to 40% of said copolymer and correspondingly from 70 to 60% of said resin and from 30 to 40% of diatomaceous earth; in said rail members from 30 to 45% of said co-

polymer and correspondingly from 70 to 55% of said resin and from 30 to 45% of diatomaceous earth; in said studs from 35 to 40% of said copolymer and correspondingly from 65 to 60% of said resin, and from 35 to 40% of diatomaceous earth; said percentages being by weight based on the sum of said copolymer and said resin.

7. A plating barrel comprising a pair of end members forming the ends of the barrel, a plurality of foraminous panels held longitudinally between said end members and forming the sides of the barrel, a plurality of longitudinal rail members between said panels, said panels being held in recesses in said end members and said rail members, a floating freely rotatable sleeve bearing located at each end of the barrel coaxially therewith centrally of said end members, a hub located at each end of the barrel coaxially therewith centrally of said end members, said hubs being fixedly connected to said end members, said bearings freely rotatably floating inside said hubs in frictional engagement therewith, a driving gear mounted coaxially with said barrel and surrounding one of said hubs, studs fixedly securing said end members to the ends of said rail members, and studs fixedly securing said driving gear to one of said end members, said parts being composed of a heat-cured composition comprising a cashew nut shell oil-modified phenol-aldehyde resin convertible to insoluble, infusible form under the action of heat and a hardening agent, a methylene-yielding hardening agent for said resin, a rubbery copolymer of butadiene and acrylonitrile, and diatomaceous earth, the relative proportions being as follows: in said end members and in at least a major proportion of the thickness of said panels from 30 to 40% of said copolymer and correspondingly from 70 to 60% of said resin, and from 30 to 40% of diatomaceous earth; in said rail members, said bearings, and said hubs from 30 to 45% of said copolymer and correspondingly from 70 to 55% of said resin, and from 30 to 45% of diatomaceous earth; in said gear from 45 to 60% of said copolymer and correspondingly from 55 to 40% of said resin and from 40 to 55% of diatomaceous earth; in said studs from 35 to 40% of said copolymer and correspondingly from 65 to 60% of said resin and from 35 to 40% of diatomaceous earth; said percentages being by weight based on the sum of said copolymer and said resin.

8. A plating barrel assembly comprising a pair of end members forming the ends of the barrel, a plurality of foraminous panels held longitudinally between said end members and forming the sides of the barrel, a plurality of longitudinal rail members between said panels, a hub located at each end of the barrel coaxially therewith centrally of said end members, a driving gear mounted coaxially with said barrel and surrounding one of said hubs, a floating freely rotatable sleeve bearing located at each end of the barrel coaxially therewith and inside said hubs, a stationary sheave located at each end of the barrel coaxially therewith and inside said bearings, said bearings freely rotatably floating between said hubs and said stationary sheaves and in frictional engagement with said hubs and said sheaves, studs fixedly securing said end members to the ends of said rail members, studs fixedly securing said hubs to said end members, and studs fixedly securing said driving gear to the adjacent one of said end members, said parts being composed of a heat-cured composition comprising a cashew nut shell oil-modified

13

phenol-aldehyde resin convertible to insoluble, infusible form under the action of heat and a hardening agent, a methylene-yielding hardening agent for said resin, a rubbery copolymer of butadiene and acrylonitrile, and diatomaceous earth, the relative proportions being as follows: in said end members and in at least a major proportion of the thickness of said panels from 30 to 40% of said copolymer and correspondingly from 70 to 60% of said resin, and from 30 to 40% of diatomaceous earth, in said rail members, said hubs, said bearings and said sheaves from 30 to 45% of said copolymer and correspondingly from 70 to 55% of said resin, and from 30 to 45% of diatomaceous earth; in said gear from 45 to 60% of said copolymer and correspondingly from 55 to 40% of said resin and from 40 to 55% of diatomaceous earth; in said studs from 35 to 40% of said copolymer and correspondingly from 65 to 60% of said resin, and from 35 to 40% of diatomaceous earth; said percentages being by weight based on the sum of said copolymer and said resin.

14

9. A plating barrel as set forth in claim 1 wherein said panels are faced internally with a layer of said heat-cured composition in relative proportions of from 45 to 60% of said copolymer and correspondingly from 55 to 40% of said resin, and from 40 to 55% of diatomaceous earth.

FERRIS E. NEWMAN.

## REFERENCES CITED

- 10 The following references are of record in the file of this patent:

## UNITED STATES PATENTS

| Number     | Name           | Date          |
|------------|----------------|---------------|
| 15 478,630 | Newhall et al. | July 12, 1892 |
| 690,240    | Cutler         | Dec. 31, 1902 |
| 800,692    | Thorpe         | Oct. 3, 1905  |
| 1,934,461  | Hartley        | Nov. 7, 1933  |
| 2,480,022  | Hogaboom       | Aug. 23, 1949 |

## OTHER REFERENCES

- Shepard et al., Modern Plastics, pages 154-156, 210, 212, Oct. 1946.